

June 7, 1966

M. MAKANSI

3,255,064

PROCESS FOR MECHANICAL CRIMPING OF FIBERS IN SHEET FORM

Filed July 17, 1961

2 Sheets-Sheet 1

FIG. 1



FIG. 2



FIG. 3



INVENTOR

MUNZER MAKANSI

BY

*Harry P. Braddock*

ATTORNEY

June 7, 1966

M. MAKANSI

3,255,064

PROCESS FOR MECHANICAL CRIMPING OF FIBERS IN SHEET FORM

Filed July 17, 1961

2 Sheets-Sheet 2



INVENTOR

MUNZER MAKANSI

BY

*Harry C. Bradick*

ATTORNEY

1

3,255,064

**PROCESS FOR MECHANICAL CRIMPING OF  
FIBERS IN SHEET FORM**

Munzer Makansi, Wilmington, Del., assignor to E. I. du Pont de Nemours and Company, Wilmington, Del., a corporation of Delaware

Filed July 17, 1961, Ser. No. 124,616  
12 Claims. (Cl. 156—166)

This invention relates in general to nonwoven webs of fibrous elements and, more particularly, to an improved processing method for producing such nonwoven webs having superior properties.

In the following specification, and in the claims, the term "fibrous elements" is intended to include any filamentary material of the type appropriate to the textile art including any fibril, fibril, fiber, filament, thread, yarn, or filamentary structure regardless of length, diameter, or composition although, in preferred form, the invention relates particularly to synthetic organic polymeric fibrous materials and, more especially, to such materials in the form of continuous filaments.

The term "web" includes mats, batts, nonwoven pile fabrics, and other interfelted, interentangled or commingled fibrous products which may generally be described as coherent sheets of entangled fibers made without the fibers first being spun into yarns and the yarns later interlaced by weaving, knitting, braiding, or other means of yarn manipulation.

In the production of nonwoven webs of fibrous elements, a number of basic problems exist with respect to fiber distribution, retention of structural integrity, and attainment of desired properties in terms of end-use function and aesthetics. It has been the experience of those skilled in the art that the parameters in their desirable ranges, more often than not, are mutually exclusive. Attaining one object in full often seems to require missing another object completely. As a result, the nonwoven structures known in the present state of the art are the result of prudent, although not always felicitous, compromises in balancing one set of objects against another.

For example, it is desirable to produce nonwoven structures from a multiplicity of continuous filaments of synthetic organic polymeric materials, thereby taking advantage of the reduced manufacturing costs inherent in such a procedure as well as producing structures of greatly increased strength and having other useful and distinctive properties. The copending application of Kinney, S.N. 859,614, filed December 15, 1959, and now abandoned sets forth a process of distributing continuous filaments to form a web composed of fibrous elements disposed in random nonparallel arrangement.

To impart certain appropriate aesthetic properties to nonwoven structures, notably soft hand and good drape, it has been found desirable to highly crimp the individual fibrous elements as set forth in the copending application of Guandique, et al., S.N. 859,640, filed December 15, 1959, and now Patent No. 3,117,055. However, it also has been found that imparting the desired high crimp to the individual elements prior to distribution in the web interferes with such distribution and, while processes for producing in situ the desired crimp level have been found, as set forth in the reference applications, a simple, effective, and inexpensive process employing largely mechanical means has not been known prior to this present invention. Attempts to act upon the entire web structure by the known processes for mechanically indenting complete matted fibrous pads and the like have not resulted in nonwoven structures in which substantially all the individual fibrous elements have a high degree of

2

crimp and have soft hand and good drape. The results of attempts to use the known art have been either a low crimp, mostly confined to the surfaces, where crimping forces were of a low order—or a crimped product, excessively stiff, where higher forces were used. In addition, the products of the prior art have been characterized by a low degree of uniformity.

It is an object of the present invention to provide an improved process for treating a nonwoven web of uncrimped fibrous elements to produce a nonwoven structure of uniformly highly crimped fibrous elements having soft hand and good drape.

Further, it is an object to treat such a web by simple, inexpensive, and largely mechanical means.

Additionally, it is an object to crimp in situ, and to a relatively high level of crimp, substantially all of the fibrous elements in a nonwoven web of randomly distributed uncrimped fibrous elements.

Yet another object is to provide a process for treating a nonwoven web of randomly distributed uncrimped continuous filamentary fibrous materials of synthetic organic polymeric material to produce a high and uniform level of crimp in situ.

It is yet another object of this invention to provide an arrangement for treating a nonwoven web of randomly distributed uncrimped fibrous materials of synthetic organic polymeric material, said web having bonding material therein, to produce a bonded nonwoven structure of highly crimped fibrous elements.

Further objects and advantages will be apparent from the description hereinafter.

In accordance with this invention the objects are attained by a process for producing a nonwoven structure of highly crimped fibrous elements preferably of synthetic organic polymeric materials and still more preferably of continuous filaments, comprising partially drawing fibrous elements and forming a web of these elements, disposed in uncrimped random nonparallel arrangement, and subjecting this web to compressive and shearing forces in a multiplicity of spatially distributed areas distributed upon at least one of the surfaces of the web, the forces being of sufficient magnitude to further draw the individual fibrous elements locally and crimp them to a high crimp level, and simultaneously heating the web uniformly and sufficiently to facilitate crimping and set the fibrous elements and then optionally, where, ordinarily, suitable binder material has been distributed in the web, subjecting the thus-drawn and crimped web to heat to produce a bonded nonwoven structure, and, optionally, embossing the surface thereof to provide further aesthetic properties.

The present invention is described in further detail below in connection with the accompanying drawings in which:

FIGURE 1 is a flow sheet of a preferred process according to the invention,

FIGURE 2 is a flow sheet of an optionally preferred process according to the invention,

FIGURE 3 is a diagrammatic representation of apparatus arranged in a system for processing articles under the principles of the invention,

FIGURE 4 is a view in projection of an enlarged fragmentary portion of a crimping surface used in practicing the process of the instant invention,

FIGURE 5 is a top-plan view of an enlarged fragmentary portion of a preferred crimping surface, and

FIGURE 6 is a side view in cross section on line 6—6 of FIGURE 5.

FIGURE 7 is a diagrammatic representation of apparatus arranged in a preferred system for further processing webs mechanically crimped according to the invention to produce an improved bulked, embossed and bonded product.

Referring to the drawings, FIGURE 1 is a flow sheet of the process for practicing the invention. From a source of fibrous elements 1, the elements are forwarded and partially drawn 2 in a uniform manner, and then forwarded to the forming step 3 in which there is laid down a web of randomly distributed uncrimped fibrous elements. This web is then forwarded to the crimping and setting step 4 wherein the web is subjected to compressive forces in a multiplicity of spatially distributed compressive areas, disposed upon at least one of the surfaces of the web, these forces selectively being of sufficient magnitude to locally draw the individual fibers to a high state of crimp. Meanwhile, the web is uniformly heated to a level sufficient to facilitate crimping and set the fibrous elements while undergoing the crimping action. This process produces a coherent web in which the individual fibers are highly crimped, the entire structure having aesthetic properties of soft hand and exhibiting a high degree of drape.

Where it is desired to produce a web structure having softness and drape with good retention of properties, it is known to bind the final structure by any one of a number of well-known means. To achieve such a product, the process of FIGURE 2 may optionally be used, in which there is withdrawn from a source of fibrous elements 1' and a binder material 1'', which later may be liquid, particulate, or preferably fibrous in form, sufficient materials and in appropriate proportions, and these are forwarded through drawing step 2' wherein the fibrous elements are drawn partially, as before. The fibers so treated thence are forwarded to process step 3' in which there is formed a web, as before, nonwoven and of randomly distributed uncrimped fibrous elements, which web is forwarded to process step 4' in which the elements are crimped and set, the crimping forces and temperatures being selected so that bonding does not occur during this process step. The material then, in the form essentially of the product of the process of FIGURE 1 with the exception of the binder material distributed therein, is forwarded to process step 5 in which bonding occurs by any of the known methods, as will be set forth in greater detail further on in this specification. It is also possible to self-bond webs of thermoplastic materials having no binder therein by appropriate adjustment of the bonding conditions, as is well known.

Referring now to FIGURE 3 in which is shown a schematic arrangement of apparatus elements adapted to producing products by processes of either FIGURE 1 or FIGURE 2 numerals 6 and 6' are representative of sources of fibrous elements and binder in the form of fibrous elements respectively. Sources of fibrous elements 6 and 6' may be spinning heads of any of the well-known types adapted to the continuous spinning of filamentary materials, and, to a person versed in the art, it will be apparent that associated equipment requisite to the proper functioning of such spinning heads and dependent upon the particular chemical and physical nature of the filaments spun are not indicated in the present schematic drawing.

As described more fully in the application of Kinney previously referred to, filaments 7, the product from source of fibrous elements 6 and filaments 8, the product from source of binder elements 6' are combined over rotatable target 9 and thereabouts charged to a suitable level of static electricity by means of source of charging 10 which may be a corona discharge or alternatively may be a contacting source of triboelectric energy or may be field charging. Thence, charged filaments 11 are passed to drawing device 12 which may be any of the known types of drawing mechanisms but preferably an air jet device as schematically indicated. Charged filaments 11 are then deposited upon moving belt 13 in an appropriate manner to form a nonwoven web 15 in which the uncrimped fibrous elements are disposed in random non-parallel arrangement.

Moving belt 13 may be foraminous or not, as appropriate to the particular product handled and, as described in the Kinney application, may be grounded electrically or oppositely charged by means of electrical device 14. The web 15 so formed moves in the direction of the arrow 5 on belt 13 and may optionally be consolidated to facilitate handling. This consolidation may be accomplished by pressing web 15 as it is carried on belt 13 between lightly loaded presser roll 16 and the downstream drive roll 17 of belt 13. Greater consolidation may be obtained by further passing web 15 through the nip between downstream drive roll 17 and the second consolidation roll 18 which ordinarily would be more heavily loaded than roll 16, and still further consolidation may take place 10 in a third nip point between roll 18 and roll 19 which latter roll may be heated if this requirement is appropriate. Web 15 may then be passed to a windup device, not shown, and a package wound up in any manner known to the art for transportation to further processing, or, as is shown in the schematic of FIGURE 3, passed, along path 20 44 shown as a dotted line, in a continuous manner around guide roll 20 to mechanical crimping device 21 passing through cooling lips 45. Cooling lips 45 are connected to a source of cooling liquid, not shown, which liquid is circulated internally entering and leaving through ports 25 46 and 47. In mechanical crimping device 21, web 15 is passed between the nip of rolls 22 and 23. Means for applying and regulating the loading in this nip, and in the other nips of the figure, are provided but not shown. Roll 23 is shown as having an elastomeric cover 24 thereon, and roll 22 is so disposed as to provide a multiplicity of compressive forces spatially distributed upon one of the surfaces of web 15. It is apparent that this may be done by providing the surface of roll 22 with some form of tessellation in which protuberances which may be pegs and clear areas alternated according to an appropriate pattern. A form of such a surface is shown in projection in FIGURE 4, which is representative of a small enlarged portion of the surface of roll 22. The pattern is shown uniformly distributed upon the surface 30 24 of the roll as a multiplicity of pyramidal pegs 25 of depth D and pitch spacing P. It should be noted here that the uniform pitch spacing P of FIGURE 4 is not a requisite of the invention, although it is a preferred form, and that other spacings may suggest themselves to practitioners of the art for achieving purposes common to that practice. Similarly, pegs 25 might well be disposed upon moving belts rather than upon surfaces of rolls such as roll 22, and still further, intermeshing rolls might be employed as the equivalent of opposing roll 22 by elastomeric covered roll 23. Furthermore, other forms of pegs or protuberances, screens for example, may be used. Experience will suggest other variations of elements that will be equivalent to the basic process herein disclosed. 35 Experience has shown, for example, that a number of crimping operations may be requisite, and hence there is indicated in the schematic of FIGURE 3 a second crimping operation between rolls 23' having elastomeric cover 24' and roll 22', the rolls being disposed on diametrically opposite sides of web 15 as compared to rolls 22 and 23. 40 A preferred crimping surface is shown in FIGURES 5 and 6. Pegs 40 have peaks 41 formed of truncated spheres. Similarly, the roots 42 are semi-circular in cross section while the flanks 43 are planar, tapering inward from root 42 to peak 41. The pitch to depth ratio of this surface is 1:1. The surface of FIGURES 5 and 6 has been found to provide more uniform properties in the end product and is particularly useful in minimizing anisotropic characteristics. 45 The process of the instant invention requires that simultaneously with the application of pressure in spatially distributed compressive areas, there be supplied heat of a sufficient magnitude to facilitate crimping and set the crimp. The elevated temperature also limits static electricity which otherwise produces a web which is too lively 50 55 60 65 70 75

and fuzzy to further handle. Thus, mechanical crimping device 21 is shown with cover 26 and heating device 27. In practice, a number of heating means may be employed to achieve the desired result, providing appropriate quantities of heat are supplied and their distribution and level is controlled properly. For example, rolls 22 and 23 may be internally supplied with steam heat, or alternatively, convectors may be used or similar devices within enclosure 26, or heating device 27 may be any of a number of known radiant heating devices heating either the surface of the roll or the surface of web 15 or both, or further, any combination of these means or other well-known means might be used to supply uniform heat in a controlled fashion to web 15 as it passes through the nip of rolls 22 and 23.

Where it becomes desirable in terms of end-use for the web to be bonded, web 15 is preferentially forwarded through cooling lips 48 to bonding and embossing device 28 which is appropriately enclosed within covering structure 29. Cooling lips 48 are appropriately connected to a circulating cooling-liquid system, not shown, by ports 49 and 50. Advancing web 15 is carried into the nip between processing belt 30, which is driven in the direction of the arrow, and heated roll 31, belt 30 being backed up at the nip by roll 32. Processing belt 30 is partially wrapped about the periphery of heated roll 31 and maintained in that position by rolls 32, 33, and 34, and belt 30 is urged against roll 31 by appropriate means not shown in the drawing. Within the nip between belt 30 and heated roll 31, web 15 is heated to a level sufficient to activate the binder material, which results in discrete bonding. If then it is desired to impart an aesthetically appealing surface pattern, web 15 is then preferentially forwarded into the nip between embossing rolls 35 and 36, which are urged one against the other, by means not shown in the drawing, with a force sufficient to indent the surfaces of the web while the binder elements may or may not be still activated to fix the surface as desired. Rolls 35 and 36 may be similar to roll 22 in formation or could be foraminous metallic structures such as screens or, without departing from the teachings of this invention, could be a combination of a deeply profiled roll with a roll having an elastomeric or similar yielding surface. Embossing rolls 35 and 36 may be internally heated and, for reasons of temperature control, may be enclosed separately from covering structure 29. Between roll 33 and the nip between rolls 35 and 36 there may be an intermediate enclosure, separately temperature controlled, to regulate the temperature gradient therebetween. Web 15 is then forwarded to a windup device, not shown on the sketch, where it is wound into a package 37 upon core 38. To insure appropriate heat transfer conditions in bond embossing device 28, suitable heating devices, indicated schematically in the drawing by heating device 39 may be employed. In addition to direct heating of roll 31, similar direct heating of rolls 35 and 36 may be required or desired. Similarly, enclosure 29 may be insulated or supplied with a heating jacket. Furthermore, the order of processing through bonding and embossing device 28 is a matter of skilled choice, and, as will be apparent to those conversant with the art, it may be more appropriate to emboss between rolls 35 and 36 prior to bonding between belt 30 and heated roll 31.

Where it becomes desirable in terms of end-use for the bonded and embossed web to have exceptional bulk, the process outlined in FIGURE 7 may be employed. Having been spun, laid down, consolidated, stabilized, and mechanically crimped in a manner according to that shown in FIGURE 3, the web emerging from mechanical crimping device 21 and shown in FIGURE 7 as 15' is passed to a mechanical working device 92 wherein at ambient room temperature web 15' is squeezed between screen roll 69 and elastomeric covered roll 70. Screen roll 69 is covered with a relatively coarse mesh screen 71

and screen 71 is urged by biasing means not shown acting on roll 69 against web 15' which is backed up by a moderately soft elastomeric cover 72 surfacing roll 70. Web 15' is then carried into embossing device 73 wherein at 5 elevated temperature an appropriate embossing pattern is placed upon the surfaces of web 15', as the web passes into the nip between rolls 74 and 75 which are biased one against the other by means not shown and whose surfaces are appropriately patterned or ornamented or the like. Embossing device 73 is appropriately heated, schematically indicated in FIGURE 7 by electrical heating device 76 although any of the known equivalents might be used, and embossing device 73 is appropriately enclosed as indicated by enclosure 77. The elevated temperature in embossing device 73 is maintained below the critical temperature at which fiber to fiber bonding will occur. Web 15', emerging from embossing device 73, is carried into bonding device 78, passing into a mild nip between belt 79 and belt 80, both of which belts move 10 in the direction of the arrows. Belts 79 and 80 may be fabricated from metal screen or asbestos cotton cloth or the like, as is well known. Belt 79 passes from roll 85 around the periphery of heated roll 82 and then over roll 87 and under tensioning roll 86 which, by means not 15 shown, may be biased in a manner regulating tension in belt 79. Belt 80 passes over roll 81 and then is carried over the arcuate surface of heat transfer device 88, which latter, by means not shown, may be appropriately heated. Thence belt 80 passes around heated roll 82 and over 20 the arcuate surface of heat transfer device 89 which may be heated or cooled by means not shown, and belt 80 is then turned around roll 83 and around biasing roll 84 which by appropriate means may be properly tensioned as indicated schematically by the weight W in FIGURE 7. In bonding device 78 the temperature that the web achieves is regulated by appropriate heat input to heat transfer devices 88 and 89 and roll 82. Herein the temperature is so regulated that the binder material is activated and, upon emerging into a cooler zone or in 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920

inch and more usually in the range of 10-100 crimps per inch and having a gross displacement transverse to the fiber axis of from 0.003 inch to 0.125 inch. In addition to this structure, observation under a microscope shows indication of a microcrimp structure. This apparently results from high contact forces at cross-over points of fiber on fiber. The frequency of the microcrimps is in excess of 130 crimps per inch, and the amplitude of the microcrimps is relatively shallow as would be expected from the impression or indentation of one fiber on another fiber. The microcrimp contributes to drape by reduction of the effective bending modulus of the individual fibers through indentations at a multitude of points along the fiber length. The macrocrimp, in itself however, produces the desired properties and results from following the process of the invention. As set forth previously, the crimp level is desired to impart flexibility to webs without sacrificing strength and other physical properties.

10 Webs, according to this invention, are characterized by having tensile strength in excess of 5 lb./in./oz./yd.<sup>2</sup>, tongue tear strength in excess of 0.7 lb./oz./yd.<sup>2</sup>, and a vibration modulus not in excess of 3000 p.s.i.

15 Vibration modulus is a measure of web stiffness. It is determined in a dynamic test involving measurement of the resonance frequency of a strip of the material when subjected to a forced vibration. The sample is clamped at one end to a sinusoidally oscillating support and the frequency in cycles per second at maximum amplitude of vibration is measured either by an oscillograph or some 20 counting device. The modulus is then calculated from the formula:

$$V.M_i = \frac{224PC^2L^4}{t^2}$$

25 where  $V.M_i$  is the vibration modulus in pounds per square inch,  $P$  is the density in grams per cubic centimeter,  $C$  is the observed frequency at resonance in cycles per second,  $L$  is the sample length in inches, and  $t$  is the sample thickness in mils. The lower the modulus, the more flexible the sample.

30 Nonwoven webs having such extreme flexibility and strength are useful in such fields as protective coverings and in upholstery when in combination with vinyl and the like, and in fields presently restricted to woven fabrics.

35 It has also been indicated previously that attempting to obtain a high level of crimp by the known method of pressing raw webs composed of undrawn fibers between plates or in calender-type rolls results in failure. Structures achieved by this approach are excessively stiff and unsatisfactory and not suitable for many fields in which more expensive woven fabric base materials are presently used. Similarly, attempts to highly crimp webs made from fibers highly drawn to achieve high tenacity resulted in failure. Such webs are characterized by an excessive number of broken filaments. Surprisingly, it was found that, for fibers in a nonwoven web structure when randomly distributed to respond to mechanical crimping in situ without forming such a boardy or stiff structure or being damaged excessively, it is necessary that these fibers be only partially drawn in a uniform and controlled manner. At the same time it has been found that excessively low levels of drawing, as determined empirically or measured by any convenient means such as average fiber X-ray orientation resulted in unacceptable mechanically crimped nonwoven structures; for example, in working with fibers formed of polyethylene terephthalate, X-ray total orientation angles greater than 60° are excessive. X-ray total orientation angles as used herein refer to the central angle sub-tended by the arc of an X-ray diffraction from half maximum intensity to half maximum intensity. The technique is described in a paper by H. G. Ingersoll, Journal of Applied Physics, vol. 17, page 924, 1946. In addition to this, it was found that variations in the draw level of individual fibers are indicated by any measure such as orientation of the individual fibers within the web must

40 be kept within reasonable limits. For example, in working with fibers of polyethylene terephthalate, optimum results were achieved only when X-ray total orientation angles were less than 60° and not less than 20° with a coefficient of variation less than 20%. In addition, it was found that temperature conditions during crimping must be adjusted to promote setting which imparts stability in the final product. The desired crimp level and a dimensionally stable nonwoven web were achieved easily in working with polyethylene terephthalate when crystallinity was low in the raw web and when temperature conditions during crimping were sufficient to induce substantial crystallinity.

45 Crystallinity as used herein is determined by X-ray diffraction techniques. The X-ray diffraction pattern of the sample is prepared by standard film techniques, using a vacuum camera, and an equatorial densitometer scan (perpendicular to the longitudinal axis of the structure) of the pattern is made. Using polyethylene terephthalate as an example which is well known, the resulting curve exhibits three peaks, corresponding to the scattering from the 010, 110, and 100 diffraction planes, which represent the principal scattering from linear terephthalate polyester crystallites. For convenience in reporting results, an arbitrary subjective rating scale has been adopted in which zero crystallinity, a totally amorphous material, is rated as 0, and the most crystalline sample recorded and known to the laboratory is rated as 9. There is thus a direct correlation with the more precise method of estimating percent crystallinity well known in the art.

50 Because of the differences between batch processing using flat plates and continuous processing using calender type rolls, particularly with regard to time-temperature relationships, it has been found appropriate in working with polyethylene terephthalate to use a higher draw in the latter case and, hence, have greater orientation and crystallinity in the fibers of the webs before crimping. Such webs, if heated while unrestrained, shorten and narrow excessively and generally shrink in a manner difficult to control. This shrinkage is minimized by preventing heating of the web while unrestrained. This, referring again to FIGURE 3, is accomplished by cooling lips 45 and 48 which are installed at the respective entries of mechanical crimping device 21 and bonding and embossing device 28.

55 Alternatively, and preferably, the minimization of shrinkage of the web, which also is termed stabilization, may be accomplished in a continuous manner by routing web 15, as it leaves roll 19, to felt calender 51 as is shown in solid lines in FIGURE 3. Prior to entering felt calender 51, web 15 is interleaved between cotton belts 52 and 53 which may be fabricated from a 72 x 72 greige cloth and move in the direction of the arrows. Web 15, so interleaved, is then carried between the surfaces of felt belt 54 and heated can, or cylinder 55, which move in the direction of the arrows. Felt belt 54 passes endlessly about rolls 56, 57, 58, 59, 60, and 62 and by tensioning means not shown is maintained in intimate contact under controlled pressure with can 55. Roll 60 is appropriately cooled by means not shown to prevent overheating of felt belt 54. Cotton belt 52 passes endlessly about rolls 63, 56, 57, 64, 65, 66, and 67 and is tensioned against can 55 by means not shown. Cotton belt 53 passes endlessly about rolls 68, 56, and 57 and is tensioned against can 55 by means not shown. As with other devices of the schematic of FIGURE 3, driving means are not shown. After stabilization in felt cylinder 51, web 15 is directed over roll 20' to mechanical crimping device 21 and proceeds as previously described except that cooling lips 45 and 48 may be inoperative without affecting web shrinkage. Treatment in a device such as felt calender 51 has been found effective in stabilizing webs and the treatment has been found to increase crystallinity of polyethylene terephthalate. Not only are subsequent tendencies to shrinkage substantially eliminated, but any subsequent

tendency to form weak fiber to fiber bonds under pressure during crimping are minimized as well as is any predisposition to mechanical damage under the action of the pegs.

Furthermore, there have been found relationships between the pitch  $P$  of the crimping surface, the groove depth  $D$  of the crimping surface, and the maximum nonwoven web weight  $W_{max}$  for each stiffness level of product. These relationships are set forth in the following formulae:

- (1)  $D \geq .3P$
- (2)  $D \geq cP + d$
- (3)  $P \geq aW_{max} - b$

where  $D$  = depth in inches,  $P$  = pitch in inches,  $W_{max}$  = basis weight in oz./yd.<sup>2</sup> and, where  $a$ ,  $b$ ,  $c$ , and  $d$  are constants, which must be determined experimentally and result from the physical properties of the fibrous elements employed and the ambient processing conditions.

In Table I are shown numerical values of constants  $a$ ,  $b$ ,  $c$ , and  $d$  for processing polyethylene terephthalate fibrous elements according to the process of this invention.

TABLE I

| Vibration Modulus (p.s.i.) | Numerical Values of Constants      |                 |                        |                 |
|----------------------------|------------------------------------|-----------------|------------------------|-----------------|
|                            | $a$<br>(in.-yd. <sup>2</sup> /oz.) | $b$<br>(inches) | $c$<br>(dimensionless) | $d$<br>(inches) |
| 600-----                   | 0.050                              | 0.045           | 0.33                   | 0.015           |
| 1,000-----                 | 0.050                              | 0.075           | 0.33                   | 0.015           |
| 1,500-----                 | 0.055                              | 0.110           | 0.33                   | 0.015           |
| 2,000-----                 | 0.055                              | 0.145           | 0.33                   | 0.015           |
| 3,000-----                 | 0.070                              | 0.260           | 0.33                   | 0.015           |

For example, with respect to webs of polyethylene terephthalate, using a crimping surface having pegs, or protuberances, spaced uniformly 12 to the inch (12 x 12) with a depth of about 0.045 inch, the upper limits of fabric weight having vibration moduli of 600, 1000, 1500, 2000, and 3000 p.s.i., respectively, were established at approximately 2.5, 3.2, 3.5, 4.1, and 4.9 oz./yd.<sup>2</sup> respectively.

It has been found that the relationships of Formulae 1, 2, and 3 are limited by the effect of increasing basis weight of the finished web structure of polyethylene terephthalate to values below 6½ ounces per square yard. Above 6½ ounces per square yard all patterns of the mechanical crimping means immaterial of pitch and depth produce structures with vibration moduli greater than about 10,000 p.s.i. at which level the structure may well be considered akin to paper while structures below a vibration modulus of 3,000 p.s.i. are akin to fabric, there being a transition zone therebetween.

Work with fibrous elements of synthetic organic materials other than polyethylene terephthalate has shown that the process of the instant invention is applicable. However, as workers in the field well know, the appropriate conditions for each particular material must be separately determined. Furthermore the measures of the conditions of one fiber may not apply to that of another. As an example, the invention was found to apply to polypropylene but X-ray data did not appear to be helpful in measuring the amount of partial drawing required or the proper level of heating needed to set the crimp. These conditions however were amenable to experimental determination. Thus, the invention is not to be characterized by a general measure.

The following examples illustrate specific embodiments of this invention that are not intended to be limiting and examples are given of the effect of working outside the invention.

#### Example 1

In accordance with the method of Kinney, elsewhere described and using the web spinning arrangement sche-

matically shown in FIGURE 3, nonwoven sheets were prepared comprising 92% polyethylene terephthalate and 8% of a binder fibrous element comprising an 80/20 mixture of a copolyester of ethylene glycol with terephthalic and isophthalic acid. Corona charging and draw jet conditions were adjusted so that the fibers of this web were partially drawn and distributed in random nonparallel arrangement. The raw web so prepared was subjected to mild consolidation by pressing it at 50° C. for 5-10 seconds under a pressure of 200 p.s.i. A hand sheet cut from this web was mechanically crimped by being pressed between a ¾-inch thick flat metal plate having 12 pyramidal protuberances per lineal inch, hence nominally designated a 12 x 12 plate, yielding a pitch of 83.5 mils, and having a depth of 80 mils, and an elastomeric sheet in a platen press heated to a temperature of 125° C., at a loading of 400 p.s.i., and held there for 180 seconds, during which period the actual sheet temperature was raised from room temperature to 95° C. The hand sheet was then subjected to a second mechanical crimping step, having been turned over on the same, already heated plate, using the same conditions of temperature, time, and pressure as used in the first step. The hand sheet was then bonded and embossed using a 70 x 70 mesh wire screen on one side and a 30 x 30 mesh wire screen on the other side, and employing a platen press heated to 220° C. at a pressure of 100 p.s.i. for 60 seconds, during which time the actual sheet temperature rose to 215° C. Fiber properties are shown in Table II-A. The resultant fabric structure was strong, highly uniform, and had soft hand and excellent drape. The physical and drape properties of the fabric are shown in Table II-B.

TABLE II-A (FIBER PROPERTIES)

|                           | Raw Web <sup>1</sup> | Consolidated Web | After Crimp #1 | After Crimp #2 | After Bond Embossing |
|---------------------------|----------------------|------------------|----------------|----------------|----------------------|
| Denier-----               | 2.91                 | 2.62             | 1.97           | 2.05           | 2.21                 |
| Stand. dev.-----          | 0.41                 | 0.35             | 0.15           | 0.26           | 0.31                 |
| Tensile (g.p.d.)-----     | 2.70                 | 2.99             | 3.40           | 3.06           | 3.26                 |
| Elongation (percent)----- | 172                  | 163              | 62             | 56             | 31                   |
| Modulus (g.p.d.)-----     | 17.3                 | 17.3             | 26.1           | 27.0           | 45.2                 |
| Work to break-----        | 2.33                 | 2.55             | 1.34           | 1.08           | 0.69                 |
| Density-----              | 1.3412               | 1.3416           | 1.3675         | 1.3656         | 1.3889               |
| X-Ray results:            |                      |                  |                |                |                      |
| Crystallinity-----        | near 0               | near 0           | 4              | 4              | 6                    |
| Rating <sup>2</sup> ----- | 50°                  | 60°              | 25°            | 30°            | 35°                  |
| Orientation-----          |                      |                  |                |                |                      |

<sup>1</sup> Typical birefringence measurement for a web of this type at this stage is 0.03.

<sup>2</sup> Crystallinity rating scale: Totally amorphous=0; Maximum crystallinity recorded=9.

TABLE II-B (FABRIC PROPERTIES)

|                                                      |      |
|------------------------------------------------------|------|
| Fabric weight, oz./yd. <sup>2</sup> -----            | 2.5  |
| Thickness, mils.-----                                | 14   |
| Tensile strength, lb./in./oz./yd. <sup>2</sup> ----- | 10.4 |
| Elongation at 9 lb./in., percent-----                | 27   |
| Elongation to break, percent-----                    | 69   |
| Tongue tear strength, lb./oz./yd. <sup>2</sup> ----- | 1.2  |
| Vibration modulus, p.s.i.-----                       | 1120 |
| Fabric quality-----                                  | Good |

#### Example 2

A web was prepared as in Example 1 but, to illustrate the harmful effect of too little drawing and cover conditions outside the range of the invention, with the processing conditions adjusted to provide less draw, and this web was consolidated, mechanically crimped, and bonded-embossed according to the process of Example 1. The resulting product was of poor quality and the web showed poor processing behavior characterized by sticking to the plate with the result that the operator inadvertently enlarged the area 14% in removing the web. In addition, the product showed poor strength and harsh hand. The physical properties of the fibers and the fabric are shown in Table III-A and Table III-B, respectively.

TABLE III-A (FIBER PROPERTIES)

|                      | Consolidated Web | After Crimp #1 | After Crimp #2 | After Bond Embossing |    |
|----------------------|------------------|----------------|----------------|----------------------|----|
| Denier               | 3.01             | 2.51           | 2.38           |                      | 5  |
| Stand. dev.          | .48              | .48            | .37            |                      |    |
| Tenacity (g.p.d.)    | 2.86             | 2.37           | 2.28           |                      |    |
| Elongation (percent) | 149              | 66             | 45             |                      |    |
| Modulus, Mi.         | 12.8             | 26.0           | 23.0           |                      |    |
| Work to break        | 2.10             | 0.91           | 0.69           |                      | 10 |
| Density              | 1.3401           | 1.3596         | 1.3724         |                      |    |
| X-Ray results:       |                  |                |                |                      |    |
| Crystallinity        | 0                | 2              | 4              |                      |    |
| Orientation          | >60°             | 40-60°         | 30-35°         | 35-40°               |    |
| Birefringence        | 0.017            |                |                |                      | 15 |

TABLE III-B (FABRIC PROPERTIES)

|                                                |      |  |  |    |
|------------------------------------------------|------|--|--|----|
| Fabric weight, oz./yd. <sup>2</sup>            | 2.2  |  |  |    |
| Thickness, mils                                | 12.4 |  |  |    |
| Tensile strength, lb./in./oz./yd. <sup>2</sup> | 7.0  |  |  | 20 |
| Elongation at 9 lb./in., percent               | 29   |  |  |    |
| Elongation to break, percent                   | 50   |  |  |    |
| Tongue tear strength, lb./oz./yd. <sup>2</sup> | 0.8  |  |  |    |
| Vibration modulus, p.s.i.                      | 1000 |  |  | 25 |
| Fabric quality                                 | Poor |  |  |    |

## Example 3.

A web was prepared as in Example 1, but with processing conditions adjusted to provide greater draw. This web was consolidated, and mechanically crimped and bond-embossed according to the process of Example 1. The fiber and fabric properties are shown in Table IV-A and Table IV-B, respectively.

TABLE IV-A (FIBER PROPERTIES)

|                      | Raw Web | Consolidated Web | After Crimp #1 | After Crimp #2 | After Bond Embossing |    |
|----------------------|---------|------------------|----------------|----------------|----------------------|----|
| Denier               | 2.17    |                  | 2.15           | 2.12           |                      | 40 |
| Stand. dev.          | 0.13    |                  | 0.14           | 0.21           |                      |    |
| Tenacity (g.p.d.)    | 3.10    |                  | 3.36           | 2.85           |                      |    |
| Elongation (percent) | 111     |                  | 92             | 60             |                      |    |
| Modulus, Mi.         | 32.8    |                  | 24.1           | 25.2           |                      |    |
| Work to break        | 2.0     |                  | 1.9            | 1.14           |                      |    |
| Density              | 1.3511  | 1.3554           | 1.3724         | 1.3992         |                      |    |
| X-Ray results:       |         |                  |                |                |                      |    |
| Crystallinity        | 4       |                  | 3              | 4              |                      |    |
| Rating               | 20-25°  | 20-25°           | 25-30°         | 20-25°         | 25-30°               |    |
| Orientation          | 0.071   | 0.054            | 0.104          | 0.117          |                      |    |
| Birefringence        |         |                  |                |                |                      |    |

TABLE V-A (FIBER PROPERTIES)

|                            | Raw Web | Consolidated Web |
|----------------------------|---------|------------------|
| Denier                     |         | 1.51             |
| Standard deviation         |         | 0.17             |
| Tenacity (g.p.d.)          |         | 2.97             |
| Elongation (1%)            |         | 111              |
| Modulus (g.p.d.)           |         | 19.1             |
| Work to break              |         | 1.97             |
| Density                    |         | 1.3498           |
| Yield point                |         | 0.64             |
| X-Ray crystallinity rating | 0       | 2                |
| X-Ray orientation angle    | 50°     | 30°              |

TABLE V-B (FABRIC PROPERTIES)

|                                                      | Before Washing    |                      | After Washing     |                      |
|------------------------------------------------------|-------------------|----------------------|-------------------|----------------------|
|                                                      | Machine Direction | Transverse Direction | Machine Direction | Transverse Direction |
| Fabric weight (oz./yd. <sup>2</sup> )                | 2.47              | 2.53                 | 2.50              | 2.71                 |
| Thickness (mils)                                     | 13.9              | 13.1                 | 13.5              | 14.0                 |
| Tensile strength (lb./in. per oz./yd. <sup>2</sup> ) | 8.9               | 7.9                  | 9.1               | 6.7                  |
| 9 lb./in. elongation (1%)                            | 16                | 30                   | 19                | 33                   |
| Break elongation (1%)                                | 48                | 68                   | 53                | 64                   |
| Tongue tear strength (lb./oz./yd. <sup>2</sup> )     | 0.73              | 1.0                  | 1.2               | 1.4                  |
| Vibration modulus (p.s.i.)                           | 1,020             | 560                  | 480               | 590                  |
| Quality                                              | Excellent         | Excellent            | Excellent         | Excellent            |

TABLE IV-B (FABRIC PROPERTIES)

|                                                |      |  |  |
|------------------------------------------------|------|--|--|
| Fabric weight, oz./yd. <sup>2</sup>            | 3.1  |  |  |
| Thickness, mils                                | 14.7 |  |  |
| Tensile strength, lb./in./oz./yd. <sup>2</sup> | 11.5 |  |  |
| Elongation at 9 lb./in., percent               | 17   |  |  |
| Elongation to break, percent                   | 67   |  |  |
| Tongue tear strength, lb./oz./yd. <sup>2</sup> | 1.6  |  |  |
| Vibration modulus, p.s.i.                      | 1560 |  |  |
| Fabric quality                                 | Good |  |  |

## Example 5

A web was prepared as in Example 4 but after consolidation and prior to mechanical crimping, the web was interleaved between cotton sheets and given one pass through a felt calender at 150° C. The time in the calender was 40 seconds, some additional samples having been run as controls to determine a minimum process time of 20 seconds below which adequate stabilization did not occur. Continuous crimping was performed as in the pre-

vious example but the cooling lips were not used. Bonding and embossing also was done, as in Example 4, on a platen press. Table VI shows the properties of the final nonwoven fabric.

TABLE VI

|                                                | Machine<br>Direction | Transverse<br>Direction |
|------------------------------------------------|----------------------|-------------------------|
| Basis weight, oz./yd. <sup>2</sup>             | 2.1                  | 2.3                     |
| Tensile strength, lb./in./yd. <sup>2</sup>     | 10.1                 | 10.5                    |
| Break elongation, percent                      | 58                   | 47                      |
| Tongue tear strength, lb./oz./yd. <sup>2</sup> | 1.8                  | 2.0                     |
| Vibration modulus, p.s.i.                      | 750                  | 520                     |
| Quality                                        | Excellent            |                         |

Attempts to lower the speed in crimping produced stiffer fabrics while increasing the speed reduced the crimp level. Similarly, higher temperatures produced stiffer, less acceptable fabrics.

*Example 6*

A web was prepared according to the method of Example 1 but with conditions adjusted to obtain a maximum draw. Note that this is outside the range of the invention. The fibers were spun with a ribbon-like cross section and where highly drawn having an X-ray orientation angle of 15°. 8 x 8 hand sheets were cut from this web after consolidation. These were subjected to mechanical crimping. At 625 p.s.i. loading the fibers were observed to be broken at the groove edges and did not conform to the pegs of the crimping plate. Successive trials were made reducing the crimping pressure to determine the highest loading at which breaking would not occur. This was found to be about 300 p.s.i., with other conditions according to Example 1 and here it was observed that no appreciable crimp appeared.

*Example 7*

A web, prepared as in Example 1 was mechanically crimped by pressing between a 1/8 inch square honeycomb plate and an intermeshing crimping plate containing 8 square-faced pegs per lineal inch at 150° C. and 200 p.s.i. for 2 minutes. The thus mechanically crimped fabric was then bonded and embossed between wire screens at 220° C. and 50 p.s.i. for 60 seconds, so that the domes were compressed. In this process, the fibers took on random, high amplitude, low frequency crimp. Similar results were obtained by replacing the honeycomb plate with an elastomeric sheet. The resulting fabric was soft, strong, and highly drapable.

*Example 8*

A web was prepared as in Example 4 but with 10% co-spun binder fibers. This consolidated web was also characterized by a high fiber shrinkage. A hand-sheet cut from the web was mechanically crimped, embossed, and bonded in one operation by pressing it between a 3/4-inch thick crimping plate having 60 parallel grooves per inch and a silicone rubber sheet. Both crimping plate and fabric and rubber sheet were initially at room temperature but were placed in a platen press, preheated to 200° C. and held therein for 2 minutes under a pressure of 630 p.s.i. Pressure was released, the sheet turned 90° relative to the direction of the grooves in the crimping plate, and the pressing operation was repeated. The resulting structure acquired a square weave-like pattern and the structure was characterized by being stretchable. Upon hand stretching, drapable nonwoven fabric was obtained.

*Example 9*

A web was prepared as in Example 4 but differing in that no binder fiber at all was contained. A hand-sheet cut from the web was placed between a 3/4-inch thick crimping plate having a pegged pattern spaced 50 x 50 to the inch, and a silicone rubber sheet, all being initially at room temperature.

The assembly was placed in a flat press preheated to 270°, and held there for 2 minutes under a pressure of 500 p.s.i. Pressure was released, the web turned upside down, and the pressing step repeated. The fabric resulting from this operation was found to be bonded and stretchable. Upon light stretching in both directions by hand, a drapable fabric was obtained having the following properties: Fabric weight, 1.5 oz./sq. yd.; tensile 5.2 lb./in./oz./sq. yd.; elongation at break, 26%; tongue tear strength, 1.12 lb./oz./sq. yd.; and vibration modulus, less than 200 p.s.i.

*Example 10*

15 A web was prepared as in Example 5 but after mechanically crimping and prior to embossing and bonding, the continuous web was pressed in steps momentarily in a platen press between a soft (45-50 Durometer hardness) 130 mil thick rubber sheet and an 8 x 8 mesh wire screen at room temperature (20° C.) with 200 p.s.i., then the web was turned over and pressed a second time under the same conditions. This process mechanically worked the web by opening and loosening up fragments which were highly compacted by the preceding mechanical crimping. As a result, the web became more bulky and softer without significant loss of crimp.

20 The continuous web was then embossed by pressing it in steps between two 30 x 30 mesh wire screens each backed up by a 62-mil silicone rubber sheet in a platen press at 170° C., 10 p.s.i. for 6 seconds. As a result, the web obtained a uniform screen-like pattern on both sides.

25 Finally, the continuous web, being supported by a leader fabric, was passed through hot air at 225° C. in a pin tenter. The time in the pin tenter was 60 seconds. As a result the web hand became a bonded fabric, the properties of which are exhibited in the table below.

30

TABLE VII

|                                                | Machine<br>Direction | Transverse<br>Direction |
|------------------------------------------------|----------------------|-------------------------|
| Basis weight, oz./yd. <sup>2</sup>             | 3.4                  | 3.4                     |
| Tensile strength, lb./in./oz./yd. <sup>2</sup> | 12.0                 | 7.0                     |
| Break elongation, percent                      | 57                   | 59                      |
| Tongue tear, lb./oz./yd. <sup>2</sup>          | 3.1                  | 3.6                     |
| Extensometer modulus, p.s.i. <sup>1</sup>      | 17,860               | 7,160                   |
| Quality                                        | Excellent            |                         |

<sup>1</sup> Extensometer moduli beyond 3,000 are excessively stiff.

*Example 11*

50 Nylon 66, polyhexomethylene adipamide, was spun by the method of Example 1 but without binder. Two hand-sheets were cut from the web and one was mechanically crimped according to the method of Example 1. Both were examined under the microscope and the mechanically crimped sample was observed to have developed a high level of crimp over and above the natural crimp level of the control. Comparison of the two showed the highly crimped sample to be the softer and more drapable, and further to be without the stiffness and excessive self-bonding ordinarily seen in mechanically crimped samples made from undrawn nylon yarns.

*Example 12*

55 A web was prepared according to Example 1 except that linear poly(propylene) was co-spun with 17% poly(ethylene) and conditions were adjusted to provide between 25 and 30% of normal draw, e.g., about a 2X draw. The raw web was consolidated flat between two sheets of rubber at 90° C., 400 p.s.i., for one minute. Hand sheets cut from this web were mechanically crimped with a plate grooved 30 x 30 to the inch against rubber once on each side at 90° C. and 400 p.s.i., for one minute. A hand sheet was then bonded and embossed at 130° C. and 400 p.s.i., between 40-mesh screens for two minutes. Properties of this web were as follows in Table 75 VIII.

15  
TABLE VIII

|                                           |     |
|-------------------------------------------|-----|
| Weight, oz./sq. yd.                       | 2.0 |
| Tenacity, lb./in./oz./yd. <sup>2</sup>    | 5.9 |
| Break elongation, percent                 | 97  |
| $M_i$ , lb./in./oz./yd. <sup>2</sup>      | 11  |
| Tongue tear, lb./in./oz./yd. <sup>2</sup> | 3.5 |
| Bending length, cm.                       | 3.4 |

## Example 13

A web was prepared according to the method of Example 12 except that 100% linear poly(propylene) was spun. The raw web was consolidated flat between two sheets of rubber at 130° C., 300 p.s.i., for one minute. Hand-sheets cut from this web were dipped in 4.3% solution of "Vistanex L-100" in xylene and dried to give 9% pick-up. These were then mechanically crimped once on each side with 30 x 30 grooves per inch plate against rubber at 130° C., 600 p.s.i., for 30 seconds. Samples were then flexed over a blunt edge to soften by mechanical working. Properties are given in Table IX following.

TABLE IX

|                                           |     |
|-------------------------------------------|-----|
| Weight, oz./sq. yd.                       | 2.7 |
| Tenacity, lb./in./oz./yd. <sup>2</sup>    | 8.3 |
| Break elongation, percent                 | 150 |
| $M_i$ , lb./in./oz./yd. <sup>2</sup>      | 7   |
| Tongue tear, lb./in./oz./yd. <sup>2</sup> | 3.1 |
| Bending length, cm.                       | 3.1 |

A control web on the above example, e.g., not mechanically crimped, would have a tensile strength between 8 and 10 lb./in./oz./yd.<sup>2</sup> and a bending length of 5 cm. Thus, the mechanical crimping gives the desired more flexible structure as shown by the lower bending length. Such a control web would have a vibrational modulus running around 15,000 while the vibration modulus of the above example would approximate 4,000 and that of preceding Example 12, about 2,000. X-ray data on the polypropylene examples indicate that the raw webs have X-ray orientation angles between 15 and 30° and crystallinity indices of 5 to 8 before mechanical crimping, with very little change taking place in these parameters as a result of the crimping operation.

## Example 14

A two denier per filament tow of poly(ethylene terephthalate) is prepared according to standard commercial practice except that the draw ratio during the washing and drawing step is reduced so that only a partial draw is accomplished. After partial drawing, the tow is not crimped, but dried and cut into staple length fibers approximating 1/4 inch long. These are blended 80/20 with fibrils of polyester prepared according to teachings of Example 142 of copending application S.N. 788,371, now U.S. Patent No. 2,999,788, and water-laid on a screen to prepare a waterleaf of randomly arranged fibers as further taught in that example. The waterleaf is mechanically crimped, bonded and embossed as in Example 1 to produce a soft, drapable, nonwoven fabric having crimped fibers between bond points and exhibiting good properties. Similarly, a tow of partially drawn poly(ethylene terephthalate) is cut into 1-inch long staple and blended with 10% of 1-inch staple fibers cut from an 80/20 mixture of poly(ethylene terephthalate)/poly(ethylene isophthalate). Both Garnett carding and Rando-webbing techniques are used to prepare webs which are crimped, bonded, and embossed as before to produce satisfactory soft, drapable, nonwoven structures.

## Example 15

A web is prepared as in Example 1 except that 90% of poly(ethylene sebacate) is spun and the 10% co-spun binder is a copolymer of 55/45 poly(ethylene terephthalate)/poly(ethylene sebacate). The subsequent mechanical crimping, bonding, and embossing process is,

as in Example 1, a soft, drapable, nonwoven structure is the result.

Similar results are obtained when the sheet is formed of filaments of poly(hexahydro-p-xylylene terephthalate) and the above mentioned co-spun binder.

In addition to the advantages heretofore cited in the specifications and examples, the process has also revealed a surprising result in making the physical properties of the crimped fibers within a given web more uniform as well as making the properties of initially different webs more uniform in the crimped in situ state. This result is shown in Table X.

15  
TABLE X  
EFFECT OF PROCESS ON PROPERTIES

| Property                  | Web Identification                                                                                                                | Initial Web                                          | Web After Two Crimpings                              |
|---------------------------|-----------------------------------------------------------------------------------------------------------------------------------|------------------------------------------------------|------------------------------------------------------|
|                           |                                                                                                                                   | Arithmetic Mean                                      | Standard Deviation                                   |
| Denier                    | (1) E74-5-NP1069-64 #13<br>(2) E74-5-NP1069-64 #16<br>(3) E60-5<br>(4) 212-T<br>(5) 11/16/1-YZ<br>(6) E74-25-5<br>(7) 11/16/3-YZ  | 2.79<br>2.98<br>2.17<br>1.51<br>1.50<br>2.86<br>2.04 | 2.52<br>2.03<br>2.12<br>1.44<br>1.30<br>2.09<br>1.22 |
| Denier Standard Deviation | (1) E74-5-NP1069-64 #13<br>(2) E74-5-NP1069-64 #16<br>(3) E60-5<br>(4) 212-T<br>(5) 11/16/1-YZ<br>(6) E74-25-5<br>(7) 11/16/3-YZ  | 0.45<br>0.20<br>0.13<br>0.17<br>0.15<br>0.41<br>0.36 | 0.20<br>0.17<br>0.21<br>0.21<br>0.09<br>0.31<br>0.08 |
| Tenacity, g.p.d.          | (1) E74-5-NP1069-64 #13<br>(2) E74-5-NP1069-64 #16<br>(3) E60-5<br>(4) 212-T<br>(5) 11/16/1-YZ<br>(6) E74-25-5<br>(7) 11/16/3-YZ  | 2.87<br>2.55<br>3.10<br>2.97<br>3.28<br>2.65<br>2.87 | 2.90<br>3.04<br>2.85<br>3.23<br>3.24<br>3.06<br>3.33 |
| Elongation, percent       | (1) E74-5-NP1069-64 #13<br>(2) E74-5-NP1069-64 #16<br>(3) E-60-5<br>(4) 212-T<br>(5) 11/16/1-YZ<br>(6) E74-25-5<br>(7) 11/16/3-YZ | 161<br>149<br>111<br>111<br>107<br>142<br>108        | 50<br>83<br>60<br>45<br>54<br>53<br>51               |
| Modulus, $M_i$            | (1) E74-5-NP1069-64 #13<br>(2) E74-5-NP1069-64 #16<br>(3) E60-5<br>(4) 212-T<br>(5) 11/16/1-YZ<br>(6) E74-25-5<br>(7) 11/16/3-YZ  | 17.9<br>17.0<br>32.8<br>19.1<br>22.1<br>15.9<br>20.8 | 26.0<br>23.6<br>25.2<br>24.0<br>23.0<br>24.6<br>28.0 |
| Work to Break             | (1) E74-5-NP1069-64 #13<br>(2) E74-5-NP1069-64 #16<br>(3) E-60-5<br>(4) 212-T<br>(5) 11/16/1-YZ<br>(6) E74-25-5<br>(7) 11/16/3-YZ | 2.36<br>1.90<br>2.00<br>1.79<br>2.00<br>1.86<br>1.71 | 0.86<br>1.39<br>1.14<br>1.00<br>1.17<br>1.03<br>1.15 |
|                           |                                                                                                                                   | 1.95<br>1.20<br>1.11<br>1.0                          | 1.11<br>1.11<br>1.11<br>1.11                         |

TABLE X—Continued

| Property     | Web Identification                                                                                                                                                  | Initial Web                                                                            | Web After Two Crimpings                                            |
|--------------|---------------------------------------------------------------------------------------------------------------------------------------------------------------------|----------------------------------------------------------------------------------------|--------------------------------------------------------------------|
| Density..... | (1) E74-5-NP1069-64 #13.....<br>(2) E74-5-NP1069-64 #16.....<br>(3) E60-5.....<br>(4) 212-T.....<br>(5) 11/16/1-YZ.....<br>(6) E74-25-5.....<br>(7) 11/16/3-YZ..... | 1.3430<br>1.3454<br>1.3511<br>1.3724<br>1.3498<br>1.3682<br>1.3520<br>1.3750<br>1.3478 | 1.3705<br>1.3580<br>1.3580<br>1.3724<br>1.3682<br>1.3750<br>1.3784 |
|              | Arithmetic Mean.....                                                                                                                                                | 1.3483                                                                                 | 1.3696                                                             |
|              | Standard Deviation.....                                                                                                                                             | .0035                                                                                  | .0057                                                              |
|              | Percent Coefficient of Variation.....                                                                                                                               | .3                                                                                     | .4                                                                 |

In the drawings and specification, there has been set forth preferred embodiments of the invention and, although specific terms are employed, they are used in a generic and descriptive sense only and not for purpose of limitation. The scope of the invention is defined in the claims.

I claim:

1. A process for producing an improved non-woven structure having a high degree of drapability and softness of hand suitable for textile fabric uses, said process comprising in combination, the steps of arranging a plurality of partially drawn fibrous elements, capable of sustaining further drawing, in a random, non-parallel arrangement to form a web, subjecting the web at least one time to compressive and shearing forces in a multiplicity of areas substantially evenly distributed over at least one of the surfaces of the web by contact of said web in a direction substantially normal to the planar axis of said web with spaced, individual protuberating elements having a frequency of occurrence of at least about 10 per linear inch, the said protuberating elements being under pressure, the forces controlled in magnitude, direction and points of application so as to crimp and further locally draw the individual fibrous elements to a macrocrimp level of at least about 10 crimps per inch, and simultaneously heating the web uniformly to a sufficient degree to facilitate the crimping action and set the fibrous elements in the crimped configurations.

2. The process of claim 1 in which the high level of crimp is indicated by a macrocrimp having from about 10 to about 100 crimps per inch with a microcrimp supercrimped thereon and having at least 130 crimps per inch.

3. The process of claim 2 in which the crimped configurations of the macrocrimp have a gross displacement transverse to the fiber axis of from 0.003 inch to 0.125 inch.

4. The process of claim 1 which further comprises arranging a suitable binder material in substantially evenly interspersed relation with said plurality of fibrous elements during formation of said web, and, subsequently to said step of setting said fibrous elements subjecting the web of crimped set fibrous elements to a treatment which bonds said elements together at a plurality of distributed points through the web.

5. The process of claim 4 in which the fibrous ele-

ments comprise continuous filaments of a synthetic polymeric composition.

6. The process of claim 5 in which said filaments are of a linear polyester composition.

7. The process of claim 6 in which said linear polyester composition is poly(ethylene terephthalate).

8. The process of claim 7 in which the partially drawn fibrous elements before crimping have been drawn to an extent indicated by X-ray total orientation angles less than about 60° and greater than about 20° and exhibit a crystallinity rating of between about 0 and 4.

9. The process of claim 4 which further comprises subjecting predetermined portions of said web to distorting forces sufficient to permanently indent said web at said predetermined portions whereby embossing of said web is effected.

10. The process of claim 1 which further comprises introducing into said web a binder material, and then subsequent to the steps set forth in claim 1 heating said web to activate said binding material whereby bonding of said web is effected.

11. The process of claim 10 in which said fibrous elements comprise continuous filaments of synthetic polymeric composition.

12. The process of claim 11 which further comprises subjecting predetermined portions of said web to distorting forces sufficient to permanently indent said web at said predetermined portions whereby embossing of said web is effected.

#### References Cited by the Examiner

##### UNITED STATES PATENTS

|           |         |               |           |
|-----------|---------|---------------|-----------|
| 2,036,838 | 4/1936  | Taylor        | 57—34     |
| 2,216,142 | 10/1940 | Taylor et al. | 28—72     |
| 2,430,868 | 11/1947 | Francis       | 156—34    |
| 2,457,784 | 12/1948 | Slayer        | 156—376   |
| 2,856,323 | 10/1958 | Gordon        | 161—165 X |
| 2,874,446 | 2/1959  | Sellers       | 28—72     |
| 2,917,806 | 12/1959 | Spence et al. | 264—168 X |
| 2,953,187 | 9/1960  | Francis       | 156—376   |
| 3,025,202 | 3/1962  | Morgan et al. | 156—34    |
| 3,040,412 | 6/1962  | Russell       | 28—72     |
| 3,050,821 | 8/1962  | Kilian        | 264—168   |
| 3,093,444 | 6/1963  | Martin        | 264—168   |

##### OTHER REFERENCES

"Polyesters and Their Applications," Bjorksten Research Laboratories, Inc., Reinhold Publishing Corp., New York (1956).

#### References Cited by the Applicant

##### UNITED STATES PATENTS

|           |        |          |
|-----------|--------|----------|
| 2,464,301 | 3/1959 | Francis. |
|-----------|--------|----------|

##### FOREIGN PATENTS

|         |        |                |
|---------|--------|----------------|
| 816,004 | 7/1959 | Great Britain. |
|---------|--------|----------------|

EARL M. BERGERT, Primary Examiner.

DONALD W. PARKER, Examiner.

R. R. MACKEY, P. R. WYLIE, J. MATHEWS,  
Assistant Examiners.